

# UNITED STATES PATENT OFFICE.

FREDERICK C. STANLEY, OF BRIDGEPORT, CONNECTICUT, ASSIGNOR TO RAYBESTOS COMPANY, OF BRIDGEPORT, CONNECTICUT, A CORPORATION OF CONNECTICUT.

## FRICITION FACING.

1,417,779.

Specification of Letters Patent. Patented May 30, 1922.

No Drawing. Original application filed September 24, 1919, Serial No. 325,915. Divided and this application filed August 23, 1920. Serial No. 405,508.

To all whom it may concern:

Be it known that I, FREDERICK C. STANLEY, a citizen of the United States, residing in the city of Bridgeport, county of Fairfield, and State of Connecticut, have invented certain new and useful Improvements in Friction Facings, of which the following is a specification.

This application is a division of an original application filed by me, on September 24, 10 1919, Serial No. 325,915.

This invention relates to improvements in friction facings and refers more particularly to a clutch facing or brake lining adapted 15 for use in motor vehicles. The invention is directed to a novel friction facing made from felted unwoven asbestos fibre saturated with a binder.

The object of the invention is to provide 20 a friction facing having a maximum tensile strength and hardness so that it can withstand the shocks to which these facings are subjected in a motor car and also will have sufficient resistance to abrasion; while at the 25 same time it has the proper coefficient of friction. It is also necessary that the binder in these facings must be unaffected by oil or water in use, which object is accomplished by the present invention without in any way 30 detracting from the other characteristics.

The process for making these friction facings may be carried out as follows: Asbestos fibre, preferably the short or low grade fibre is first ground in a suitable grinding machine or cutter. The ground material is then put into a beater mixed with the water or other solution and beaten into a pulp. The pulp is then delivered to a paper making machine, as for example, a wet board machine and formed into sheets or boards of 40 suitable width and thickness. This forms an unwoven felted sheet.

As a feature of the invention, there is mixed with the pulp in the beater a sulphurizing agent, as for example, sulphur, lead sulphide or analogous sulphides. In using sulphide as a sulphurizing agent, the amount employed is approximately 1.6 per cent by the weight of the asbestos fibre although this can be varied according to the 50 characteristics of the product desired. This sulphurizing agent facilitates or hastens the cure of the binder and adds to the strength

of the product and also converts the binder into a form insoluble by oil or water. It 55 also tends to produce a uniform curing throughout the mass during the curing operation hereinafter described. It is to be noted that this reagent is put into the pulp before the formation of the sheet and not 60 during the saturating and curing steps of the process.

After the sheets or boards have been formed as described, they are subjected to hydraulic pressure in suitable presses and 65 are then hung up to dry in a drying room of sufficient temperature to remove the water. The sheet is then calendered to the desired thickness, and the friction facings are then 70 cut out of the sheet. The sheets are subjected to sufficient pressure in the calender to obtain as much tensile strength in the dry sheet as is feasible. The friction facings, whether clutch rings or brake linings are now ready for saturation. The saturating 75 tank is filled with a binder. This binder may consist of 94 per cent of linseed oil, 6 per cent of gilsonite in the solution in the oil, thinned with gasoline to about 33° Baumé 80 gravity. The friction facings are then immersed while suspended on suitable rods in this binder solution for a period of half an hour. The friction facings are then removed and put in a closed steam oven and maintained at a temperature of about 200° F. to 85 drive off the gasoline, which gasoline may be recovered and saved. This steam treatment is preferably continued from two to three hours. The friction facings are then removed to a closed baking oven where they 90 are subjected to a temperature of about 250° F., for a period of twelve hours. The facings are then taken out of the oven and immersed in another saturating tank containing a solution of 66 per cent of linseed oil and 95 33 per cent of gasoline, the gravity of the solution being about 33° Baumé. This second immersion takes place for from two to three minutes. In both of the saturating steps, double boiled linseed oil is preferable. The 100 friction facings are then put into a second closed baking oven and maintained at a temperature of 300° F. for twenty four hours. The heat in both of the baking ovens is preferably dry heat. The friction facings are 105 then removed from the second oven and sand

papered to micrometer size and to get a smooth finish to the facing. The facings are now ready for use.

I have given above an illustration in 5 which the process is actually carried out in commercial operation. It is to be understood that the temperature and length of treatment are subject to reasonable variations depending on the flexibility and 10 strength required in the finished product. Also oils other than linseed oil may perhaps in certain cases be used and other asphalts substituted for gilsonite.

During the baking operation, the linseed 15 oil, due to the presence of the water in the oven and also to the sulphurizing agent of the sheet is sulphurized to produce a tough hard binder. The solubility of the linseed oil before the baking treatments is practically 20 100% in the gasoline while after the baking treatments it is very materially reduced; and in fact the baking operation may be so carried out as to make the oil practically insoluble in gasoline. It is to be noted 25 that by means of the double saturation and double baking, a more efficient curing of the binder is obtained and the sheet can be impregnated with larger quantities of binder. This adds greatly to the tensile strength and 30 hardness of the finished product.

The strength and hardness of the product made by this process is in excess of 3000 to 4000 lbs., upwards in tensile strength, over that heretofore obtained from any unwoven 35 saturated friction facing and is even stronger.

than a woven sheet. The Brinnell hardness also is proportionately increased over the friction facings heretofore made and is above 15. It is to be noted that in the baking operation, the reaction develops auto- 40 genous heat or in other words exo-thermic and care must be taken to prevent the material from becoming so highly heated as to catch fire. This exo-thermic reaction results in the fact that the sulphurization is of such 45 a character as to generate heat in addition to that externally applied. This exo-thermic reaction of sulphurization is well known in other arts, as for example, in the manufacture of air blown asphalt from petroleum 50 residuum.

I claim as my invention:

1. A friction facing composed of unwoven sheet asbestos fiber, saturated with a baked sulphurized linseed oil binder. 55

2. A friction facing composed of unwoven sheet asbestos fiber, saturated with a baked sulphurized binder.

3. A friction facing composed of unwoven sheet asbestos fiber, saturated with a baked 60 sulphurized binder, and having a Brinnell hardness in excess of ten and a tensile strength in excess of twenty five hundred.

4. A friction facing composed of unwoven sheet asbestos fiber, saturated with a baked 65 sulphurized linseed oil binder, and having a Brinnell hardness in excess of ten and a tensile strength in excess of twenty five hundred.

FREDERICK C. STANLEY.